

Mar. 6, 1923.

M. F. CHASE ET AL  
ROASTING SULPHUR BEARING MATERIALS, ETC.  
FILED MAY 1, 1919.

1,447,645.

2 SHEETS—SHEET 1.



**INVENTORS**

INVENTORS  
March F. Chase  
Frderic C. Pierce  
John Skogmark  
87  
Sexton, Jeffery Kimball & Eggleston  
ATTORNEYS

Mar. 6, 1923.

1,447,645.

M. F. CHASE ET AL  
ROASTING SULPHUR BEARING MATERIALS, ETC.  
FILED MAY 1, 1919.

2 SHEETS—SHEET 2.

Fig. 3



Fig. 4



Note.—The volumes given as 1000 cu. ft., 700 cu. ft., etc. mean rates of flow, for instance 1000 cu. ft. per minute or per hour.

INVENTORS  
March & Chase  
Edwin S. Pierce  
John Skoglund BY  
Jeffrey Kimball Venable  
ATTORNEY

## UNITED STATES PATENT OFFICE.

MARCH F. CHASE, OF CLEVELAND, OHIO, AND FREDERIC E. PIERCE AND JOHN SKOGMARK, OF NEW YORK, N. Y., ASSIGNORS TO THE COS PROCESS COMPANY, INC., OF NEW YORK, N. Y., A CORPORATION OF NEW YORK.

## ROASTING SULPHUR-BEARING MATERIALS, ETC.

Application filed May 1, 1919. Serial No. 294,065.

*To all whom it may concern:*

Be it known that we, MARCH F. CHASE and FREDERIC E. PIERCE, both citizens of the United States, residing, respectively, said 5 CHASE at Cleveland, Ohio, and said PIERCE at New York city, N. Y., and JOHN SKOGMARK, a subject of the King of Sweden, residing at New York city, N. Y., have invented the following described Improvements in Roasting Sulphur-Bearing Materials, Etc.

Sulphur dioxide ( $\text{SO}_2$ ) is produced in the process of roasting sulphide ores of zinc, iron, copper, etc., burning sulphur as brimstone or from any sulphur bearing materials 15 and is used subsequently as a gas in processes by which the said  $\text{SO}_2$  may be converted into elemental sulphur (S) liquid  $\text{SO}_2$ , sulphurous acid ( $\text{H}_2\text{SO}_3$ ) or a water 20 solution of the same, sulphuric acid ( $\text{H}_2\text{SO}_4$ ) either in a diluted form or as sulphuric anhydrid ( $\text{SO}_3$ ) or combinations for uses in the arts.

Roasting of the sulphide ores mentioned 25 is a necessary operation because it has not been found generally possible to smelt or otherwise treat metallurgically these ores until almost free of their sulphur content.

The process of roasting such ores, as usually carried on, consists in burning off the sulphur, which is accomplished in furnaces or burners of several well known types. In these, the ores, brought up to the temperature of ignition by the heat in the burner 35 gases, are rabbled mechanically continuously or intermittently or otherwise stirred and gradually made to pass through the furnace or burner, the sulphur, burning off meanwhile, deriving the oxygen necessary for 40 the combustion from the air admitted in proper quantity through adjustable openings in the furnace or burner. The product of the combustion of the sulphur,  $\text{SO}_2$ , mixes with the uncombined oxygen in the admitted 45 air, the nitrogen and other constituents present and forms the burner gases referred to above. The percentage of  $\text{SO}_2$  by volume in these gases ordinarily varies between 5% and 7%, but it may be quite low, 1% or 2%, 50 and under certain conditions quite high, 14% or 15%. In any event the strength of the gas is limited by the per cent of oxygen in the air. As it is desirable in some operations to have burner gases very rich in  $\text{SO}_2$  and to

have the percentage of  $\text{SO}_2$  under control, 55 it is one object of this invention to bring this about.

As the ore passes through the furnace, the sulphur burning off the while, the sulphur content is gradually reduced until such time 60 as it is discharged from the furnace when its content of sulphur, in the case of iron ore may be as low as 1% or even less. Such a roasted ore is said to be dead or sweet roasted. Dead roasted iron or zinc ores are 65 very necessary for satisfactory metallurgical operations such as smelting them to obtain the metals. With copper and lead ores the dead roast with present metallurgical practice is not essential. The character of the 70 ore, whether easily roasted or roasted with difficulty determines more or less the possibility of producing a dead roast without the use of external heat. By the use of heat from some other source the dead roasts required 75 may be obtained but this involves the extra expense of fuel and complications in the furnace construction. If coal is used for this purpose in connection with roasting zinc ores the amount required will vary between 5% and 35% of the weight of the ore and its cost will be one of the considerable items in the total cost of roasting such ores. 80 No way has yet been discovered to successfully use this heat in a continuously rabbled furnace without mixing the coal gases with the burner gases, which is highly objectionable if the  $\text{SO}_2$  is to be used subsequently 85 for the manufacture of liquid  $\text{SO}_2$  or  $\text{H}_2\text{SO}_4$ . Besides these there are other objections such as additional equipment, extra labor, etc. Further objects of this invention are to do away with this extra fuel and at the same 90 time produce the dead roasted ore, which will be explained presently.

The heat units generated by burning the sulphur in ores commonly treated are theoretically sufficient to roast the ore, if efficiently applied, even after reasonable allowances are made for radiation, but there are other more serious losses. The main ones are, 1st, radiation; 2nd, that carried away in the hot burner gases; 3rd, that lost in the hot roasted ore discharged from the furnace. The first can be somewhat controlled but there will be an unavoidable loss on this account even if reduced to a minimum. The third is unavoidable but is 100 105

not very great and may be recovered in ore coolers so designed as to preheat the air admitted to the furnace. The second due to the great volume of the burner gases makes 5 for the most considerable loss, although some of this may be reclaimed in a suitable air-heater. Further objects of this invention are to control the unavoidable losses and reduce them to minima and to greatly 10 limit the loss due to the large volume of the burner gases by reducing this volume.

In place of air the process employs oxygen gas or gas mixture with a higher content of oxygen than ordinary air as the principal 15 source of oxygen for burning the sulphur. In such a gas mixture the percentage of nitrogen and other inert gases in air may be exceedingly small and in any case will be less than in ordinary air. Thus the high 20 content of  $\text{SO}_2$  in the gases may be obtained by burning the ore in a furnace in which the gas mixture rich in oxygen is admitted. It is evident that the use of such a gas mixture may produce temperatures in the furnace 25 greatly in excess of those ordinarily encountered in metallurgical work and the usual construction of such furnaces might not stand up under the conditions then brought about, unless the combustion is under nice 30 regulation and complete control.

This invention relates to such regulation and complete control as applied generally to such a process and in particular to the special applications of the same for the dead 35 roasting of zinc and iron ores and for the burning of brimstone.

The process is as follows:—

A volume of gas containing any desired 40 percentage of  $\text{SO}_2$  is made to circulate in a system made up of apparatus such as the furnace or burner, a dust catcher, if necessary, following the burner, a gas cooler, which may be the dust catcher or combined with it, a blower to propel the gas, and if 45 necessary with a by-pass to control its volume, and pipe connecting the apparatus mentioned. The gas circulating in this system is enriched with oxygen by such an amount as may be necessary for the rate of 50 combustion desired, from any oxygen supply, under pressure, either in the form of oxygen gas or a gas mixture with a higher content of oxygen than ordinary air, which supply is automatically under complete control, 55 and following the burner or, if preferable, the dust catcher, if used, or the gas cooler, an equivalent amount of burner gases, now with  $\text{SO}_2$  replacing the oxygen to the extent desired is withdrawn from the system by a 60 blower or other suitable means for the purposes as previously stated, viz:—for conversion into elemental sulphur, liquid  $\text{SO}_2$ , sulphurous acid, sulphuric acid or sulphuric anhydrid, etc.

65 By varying the volume of gas circulated

the temperature of the furnace or burner can be regulated and the rate of burning the sulphur controlled. This regulation of the volume of the gas circulated is effected by the by-pass of the blower, which consists of 70 a pipe with a valve in it. By opening or closing this valve the amount of gas circulated by the blower can be controlled to a nicety. The regulation can also be accomplished by using a fan type blower with a 75 valve in the pipe.

The oxygen supply is connected up with the blower in such a way as to shut it off in case the blower stops accidentally or otherwise.

80 The rate at which the oxygen supply is admitted depends on the amount withdrawn at the exit and an automatic control is installed between the blower and the oxygen supply regulating the amount admitted, such 85 automatic control being of several types and well known.

This system of apparatus and pipes would also have the necessary valves, measuring 90 instruments for temperatures and pressures, machines to automatically analyze the gases and such other appliances ordinarily used in such combinations and is not in any way limited to the exact parts mentioned which are cited as the principal elements for the 95 purpose of a clear description.

The diagram Fig. 1, shows the system consisting of the furnace or burner (1), the gas cooler (2), the blower (3), the by-pass of the blower (4), the connecting piping (5), 100 the oxygen supply (6) the exit (7), various valves (8) measuring instruments for temperatures (9), for pressures (10), for flow of gases (11), automatic connection between exit blower and oxygen supply for control 105 of the latter (12), emergency shut off for oxygen supply (13). Such a system is adapted to the burning of sulphur or brimstone.

The diagram Fig. 2 shows a variation of 110 a part of the system in diagram Fig. 1 in that, part of the oxygen supply is introduced directly into the lower hearths of the furnace. The reason for this is to bring about a more active combustion in that part 115 of the furnace where the sulphur content of the ore has been reduced to 5% or less and thus reduce it to the minimum without bringing it in contact with gases with a high percentage of  $\text{SO}_2$ , which would interfere 120 with the desired elimination of sulphur in the ore. Such a system is adapted to the dead roasting of zinc and iron ores.

It is to be understood that in the general 125 application of this process and also in the special application it is sometimes desirable to return the circulating gas enriched with oxygen at more than one point on one hearth or on several hearths and this also applies to the introduction of the oxygen gas or gas 130

mixture with the high content of oxygen which may be introduced at several points on one or on more than one hearth. Mixture of the gases is in this case effected partly in their passage through the furnace.

It is desirable in same cases to withdraw the gases from the furnace or burner at one or more points on one hearth or on several hearths and repass all or a part thereof through one or more hearths to control the temperatures within the furnace or burner and it is to be understood that any such variations not shown in the diagrams are nevertheless to be included in this method of operation which has been described.

In roasting zinc or iron ores part of the oxygen introduced in the furnace is used to oxydize the metals and part of it used for burning the sulphur which is of course also an oxidation reaction. In this case more oxygen is introduced in the system than is removed in the exit and a relation has to be established between them. This depends on the character of the ore and the analyses of the gases and the volume circulated. Means for making this adjustment rests in the speed of the blower on the exit which is under control, and the connection between this blower and the oxygen supply.

In burning sulphur in the form of brimstone which is almost pure sulphur, practically all of the oxygen admitted unites with the sulphur to form  $\text{SO}_2$  and the volume introduced, barring leaks in the apparatus and the small percentages of impurities in the brimstone which may require a small amount of oxygen, would be the same as the volume withdrawn at the exit—reduced of course to the standard temperature of  $0^\circ \text{ C}$ . which is used in calculating gas volumes.

The foregoing operations thus bring about two general classes; first, where a considerable part of the oxygen is required for the oxidation of the ores and the gas withdrawn at the exit is considerably less than that introduced as the oxygen supply, and second, where the volume of gas withdrawn is practically the same as the volume from the oxygen supply admitted to the furnace.

The following two examples will serve to explain this in more detail.

In a zinc roasting furnace suppose the volume of gas circulating is 1000 cu. ft. (reduced to  $0^\circ \text{ C}$ ) then the volume from the oxygen supply admitted to it just before it enters the furnace, or, mixed with it inside the furnace, might be 700 cu. ft., making a total of 1700 cu. ft. In the furnace we will suppose the ores require the oxygen equivalent to 200 cu. ft. of this gas, then the gas leaving the furnace would have a volume of 1500 cu. ft. but this would have the desired analysis of the circulating volume. Of this, 500 cu. ft. is withdrawn at the exit and the balance of 1000 cu. ft. returns to the blower

and goes through the cycle again. The diagram Fig. 3, shows this condition theoretically and reference to it will show clearly the complete cycle. In practice there would be some variations from this from time to time but the means for adjusting these variations has already been explained and by use of these adjusting means a balance in the operation of the cycle may be brought about.

The diagram Fig. 4, shows how the cycle would work out theoretically when burning sulphur. The explanation of the diagram Fig. 3 and the remarks preceding it give all that can be said about this except that it will be noted that the same volume of gas (reduced to  $0^\circ \text{ C}$ ) is withdrawn at the exit as is admitted from the oxygen supply.

Comparison of these two examples will also show that in roasting ore a gas mixture is introduced in the furnace having a high percentage of oxygen for the purpose of obtaining more rapid combustion and higher temperature to roast the ores more effectively.

These examples are selected more or less at random and are cited to show the wide variations that may be brought about to suit the conditions which may have to be met.

To be more specific the point is that this process serves to control the rate of combustion in and otherwise regulate the furnace or burner and to improve the practice over what has formerly been possible both in obtaining rich  $\text{SO}_2$  gas and producing dead or sweet roasted ores and it is to be construed broadly and not limited in any way by the diagrams, which are purely for explanation purposes.

The furnace or burner herein referred to may be of the general type illustrated for example in Patent No. 916,234, or any equivalent structure.

Having thus described our process, we now claim the same as follows:—

1. A method of roasting sulphur-bearing ores of zinc, iron, copper, etc., which consists in circulating a gas mixture consisting mainly of sulphur dioxide, oxygen and nitrogen through a furnace and in contact with the ore therein, introducing oxygen to establish in the furnace a reactive medium of greater oxygen content than air, abstracting a relative portion of the mixture from the circulation and controlling the temperature of the gases circulated.

2. A method of roasting sulphur-bearing ores of zinc, iron, copper, etc., which consists in circulating a gas mixture consisting mainly of sulphur dioxide, oxygen and nitrogen through a closed system including a furnace, admitting said mixture to the furnace at different points, introducing oxygen to maintain in the furnace a reactive

medium of higher oxygen content than air, and abstracting a corresponding portion of the mixture from the system.

3. A method of roasting sulphur-bearing ores which consists in circulating a gas mixture consisting mainly of sulphur dioxide, oxygen and nitrogen through a closed system including a multiple-hearth furnace, admitting the same to different hearths of said furnace and introducing oxygen to one of said hearths to establish therein a reactive medium of greater oxygen content than air.

4. A method of roasting sulphur-bearing ores of zinc, iron, copper, etc. which consists in circulating a gas mixture consisting of sulphur dioxide, oxygen and diluent gases, through a closed system including the upper hearths of a multiple hearth furnace, introducing a gas rich in oxygen to the lower of said hearths to establish therein a reactive medium of higher oxygen content than air, abstracting from the circulation a relative portion of the increased volume, and controlling the temperature of the gases circulated.

5. The method of roasting sulphide ores or sulphur-bearing materials which consists in passing a current of gas with a higher oxygen content than air through a combustion chamber in contact with said materials, and varying the oxygen content of said gas to control the temperature of said chamber and at the same time producing a gas with a high  $\text{SO}_2$  content.

6. The method of roasting sulphur-bearing materials which consists in passing a current of gas with a higher oxygen content than air through a combustion chamber in contact with said materials and controlling the temperature in the combustion chamber by varying the flow therethrough.

7. The method of roasting sulphur-bearing materials which consists in passing a current of gas with a higher oxygen content than air in contact with a counter current of said materials and maintaining a predetermined temperature condition in the current of said materials by varying the oxygen content of said gas.

8. The method of roasting sulphur-bearing materials which consists in passing a current of gas with a higher oxygen content than air in contact with a counter current of said materials and maintaining a predetermined sulphur content of the material by varying the oxygen content of said gas.

9. A method of roasting sulphur-bearing ores, of zinc, iron, copper, etc., which consists in circulating a gas mixture consisting mainly of sulphur dioxide, oxygen and nitrogen in contact with and counter to a stream of said ore in a suitable furnace, introducing oxygen so as to establish a reactive

medium of higher oxygen content than air in the part of said furnace which is adjacent the point of ore discharge, abstracting a relative portion of the mixture from the circulation and controlling the temperature 70 of the gases circulated.

10. A method of roasting sulphur-bearing ores which consists in causing the ore to progress through a suitable furnace, circulating a gas mixture consisting mainly of sulphur dioxide, oxygen and diluent gas through a closed system including said furnace and in contact with said ore, introducing oxygen to the furnace near the point of ore discharge to establish therein a reactive medium of higher oxygen content 80 than air and regulating the temperature of the furnace by controlling the rate of flow through the system.

11. Method of producing sulphur dioxid 85 of high concentration, comprising preparing a gaseous mixture consisting essentially of sulphur dioxid and oxygen, and reacting therewith on a sulphur-bearing material.

12. Method of producing sulphur dioxid 90 of high concentration, comprising reacting on a sulphur-bearing material with a mixture containing sulphur dioxid and oxygen, the oxygen content of the mixture being in excess of the oxygen content of atmospheric 95 air.

13. Method of producing sulphur dioxid of high concentration, comprising reacting on a sulphur-bearing material with a mixture containing sulphur dioxid and oxygen, 100 the oxygen content of the mixture approximating 40%.

14. Method of producing sulphur dioxid of high concentration, comprising roasting 105 a sulphur-bearing material and withdrawing the evolved gases, adding to a portion thereof sufficient oxygen to give an oxygen concentration in excess of that of atmospheric air, and returning the oxygen-containing portion of the gases to the roasting chamber.

15. Method of producing sulphur dioxid of high concentration, comprising roasting a sulphur-bearing material and withdrawing the evolved gases; adding to a portion thereof sufficient oxygen to give an oxygen concentration approximating 40%; and returning the oxygen-containing portion of the gases to the roasting chamber.

16. Method of producing sulphur dioxid 120 of high concentration, comprising roasting a sulphur-bearing material, withdrawing and cooling the evolved gases, adding to a portion thereof sufficient oxygen to give an oxygen concentration in excess of that of atmospheric air, and returning the oxygen-containing mixture to the roasting chamber.

17. Method of producing sulphur dioxide 125 of high concentration which consists in roasting a sulphur-bearing material in a 130

- suitable furnace, abstracting some of the evolved gases, circulating the remainder through a closed system including the furnace, introducing to the system sufficient 5 oxygen to give an oxygen concentration in the furnace in excess of that of atmospheric air, and controlling the temperature of the furnace by controlling the rate of oxygen flow thereinto.
10. 18. Method of dead-roasting sulphide ores of zinc etc. which consists in passing the ore through a furnace, passing a gas mixture consisting essentially of sulphur dioxide and oxygen through said furnace in contact with the ore, introducing oxygen to that part of 15 the furnace where the ore contains less than about 5% of sulphur to establish in said part an oxygen concentration in excess of air, and regulating the furnace temperature by controlling the volume of gases passing 20 through the furnace.

In testimony whereof, we have signed this specification.

MARCH F. CHASE.  
FREDERIC E. PIERCE.  
JOHN SKOGMARK.